

## UNITED STATES PATENT OFFICE

2,189,571

## ALLOYS

Cecil Spencer Sivil, Elizabeth, and Edward O. Liebig, Arlington, N. J., assignors to Baker & Company, Inc., Newark, N. J., a corporation of New Jersey

No Drawing. Application September 13, 1939,  
Serial No. 294,646

7 Claims. (Cl. 75—172)

This application is a continuation in part of our application Serial No. 231,754, filed September 26, 1938, allowed April 5, 1939, and this invention relates in general to alloys and more particularly to alloys for use in dentures and dental appliances, for instance orthodontia wires, clasps, etc., and for jewelry and like purposes.

The prime object of our invention is to provide an alloy which shall have the color and general appearance of platinum and which shall be highly resistant to corrosion and oxidation, which shall have such ductility that it can be easily mechanically worked into suitable shapes, which shall have great hardness and high tensile strength to take and retain a high polish and to withstand stresses, particularly such as are incident to use in dental appliances, and which shall have a high temperature softening point so as to permit operations involving high temperatures, such as soldering, welding, casting other metals against it, and the like, without the great strength being lost.

We have found that alloys of platinum, palladium, silver and gold are admirably suited for the purpose with the proportions of the metals varying from 20 to 60% platinum, from 10 to 40% palladium, from 10 to 50% silver, and from 1 to 25% gold. If particularly great corrosion resistance is desired the combined content of platinum and gold should not fall below about 40% and the combined content of palladium and silver should not exceed about 60% of the total alloy, nor should the silver exceed about 35%. Alloys having from 20% to 50% platinum, from 15% to 40% palladium, from 15% to 50% silver and from 1% to 20% gold, are desirable, while when great hardness and high corrosion resistance even toward contaminated acids are desired, the following alloys are especially satisfactory:

- (1) 40% platinum, 30% palladium, 25% silver, 5% gold.  
(2) 40% platinum, 25% palladium, 25% silver, 10% gold.

Those alloys having the gold content ranging from 10% to 25% have the advantage of being practically resistant to attack by chloride compounds such as are used in dental investment compositions that are employed in casting metals, and the following alloy is recommended:

- (1) 30% to 40% platinum, 25% to 30% palladium, 20% to 25% silver and 10% to 25% gold.

Experience has shown that these preferred alloys are resistant for extended periods of time to acids contaminated with iron and materials usually occurring in pickling acids used in dental

laboratories, such as oxyphosphate cements, etc., even when in contact with other metals or alloys having a different electrical potential.

The alloys have been found to be highly resistant to corrosion and attack by acids including those acids most commonly used in dentistry, such as hydrochloric acid, nitric acid and sulphuric acid, concentrated as well as dilute.

Also they have great hardness and high tensile strength which is extremely desirable where dental appliances are subject to stresses; for example the alloy containing 40% platinum, 30% palladium, 25% silver, 5% gold has, when hard, an ultimate tensile strength of 168,000 pounds per square inch and a Rockwell hardness of 110 B 15 scale. While sufficient restoration of ductility for further working is obtained by heating below 1200° C., the alloys do not become dead soft until they have been heated above 1200° C. When heated at the lower temperatures sufficient hardness is retained to render the alloys particularly suited for appliances subject to soldering and welding operations and for appliances against which other metals or alloys are cast, especially since such operations are carried out at temperatures of 700 to 900° C. A clasp wire, for instance, may be soldered to dentures, or the dental metal or alloy may be cast against the clasp wire without danger of softening of the metal of the wire and without danger of overheating which might affect detrimentally the structure of the alloy.

It should be understood that the limited proportions above specified are not critical and that suitable alloys may be formed with the metal proportions varying more or less from the maximum and minimum limits specifically stated.

Furthermore, the alloys may also contain small quantities, for example up to a few percent, of any other metal or metals which will not deleteriously affect the fundamental characteristics of the alloys as described, such as another metal of the platinum group other than platinum and palladium, or heavy base metals or metals contributing to age hardening such as tin, zinc and cadmium.

The alloys are especially useful for dental devices that are used in the mouth, such as orthodontia wires, tooth bands, orthodontia locks, clasps, dentures and kindred devices.

Having thus described our invention, what we claim is:

1. An alloy of from twenty (20) to sixty (60) percent platinum, ten (10) to forty (40) percent palladium, ten (10) to fifty (50) percent sil-

- ver, and from one (1) to twenty-five (25) percent gold.
2. An alloy of from twenty (20) to sixty (60) percent platinum, ten (10) to forty (40) percent palladium, ten (10) to fifty (50) percent silver, and from one (1) to twenty-five (25) percent gold, wherein the combined content of platinum and gold is not less than about forty (40) percent and the combined content of palladium and silver is not more than about sixty (60) percent.
3. An alloy of about thirty (30) to forty (40) percent platinum, from about twenty-five (25) to thirty (30) percent palladium, about twenty (20) to twenty-five (25) percent silver, and from about ten (10) to twenty-five (25) percent gold.
4. An alloy composed of from twenty (20) to fifty (50) percent platinum, fifteen (15) to forty (40) percent palladium, fifteen (15) to fifty (50) percent silver, and from one (1) to twenty (20) percent gold.
5. An alloy composed of from twenty (20) to fifty (50) percent platinum, fifteen (15) to forty (40) percent palladium, fifteen (15) to fifty (50) percent silver, and from one (1) to twenty (20) percent gold, wherein the combined content of platinum and gold is not less than about forty (40) percent and the combined content of palladium and silver is not more than about sixty (60) percent.
6. An alloy composed of from twenty (20) to fifty (50) percent platinum, fifteen (15) to forty (40) percent palladium, fifteen (15) to thirty-five (35) percent silver, and from one (1) to twenty (20) percent gold, wherein the combined content of platinum and gold is not less than about forty (40) percent and the combined content of palladium and silver is not more than about sixty (60) percent.
7. An alloy consisting of about forty (40) percent platinum, from about twenty-five (25) to thirty (30) percent palladium, about twenty-five (25) percent silver, and from about five (5) to ten (10) percent gold.

CECIL S. SIVIL.  
EDWARD O. LIEBIG.

15  
10  
15  
20